

## UNITED STATES PATENT OFFICE

2,394,750

EXECUTION OF CATALYTIC CONVERSIONS  
IN THE PRESENCE OF FERROUS METALS

Robert M. Cole and Irving I. Shultz, Long Beach,  
Calif., assignors to Shell Development Company,  
San Francisco, Calif., a corporation of  
Delaware

No Drawing. Application March 28, 1942,  
Serial No. 436,618

11 Claims. (CL 260—683.3)

The present invention relates to the catalytic conversion of organic materials in the vapor phase at elevated temperatures in the presence of ferrous metals. A particular aspect of the invention relates to the treatment of hydrocarbon vapors at elevated temperatures, i. e. from about 500° F. to 1300° F., with dehydrogenation catalysts such, in particular, as those comprising an oxide of titanium, vanadium, chromium, manganese, molybdenum or tungsten, which are normally substantially free of iron and which are subject to poisoning by iron.

As is well known, one of the most common and practical methods for executing catalytic conversions of organic materials in the vapor phase is to provide a porous bed of catalyst in a suitable reaction tube, converter, or catalyst case, and to pass the vapors of the carbonaceous reactant therethrough under appropriate conditions of temperature, pressure, etc. In most cases when treating carbonaceous materials at temperatures in the order of 500° F. to 1300° F., the catalyst gradually loses its activity due to the deposition thereon of carbonaceous materials. This deactivation of the catalyst is temporary and may be indefinitely counteracted by periodically burning off the deposited materials in situ. Catalysts used in such processes, wherein they are periodically regenerated by burning carbonaceous deposits therefrom, are hereinafter referred to as regenerative catalysts.

Many of the most effective catalysts for these various conversions are susceptible to poisoning by iron. These various catalysts, when used for the vapor phase conversion of organic materials at elevated temperatures in the presence of iron, steel or ferrous alloys, besides undergoing the above-mentioned temporary deactivation due to an accumulation of carbon and tarry deposits, undergo a permanent deactivation due to the accumulation of iron or iron compounds formed by the oxidation or corrosion of the ferrous metal in contact therewith. Even traces of iron derived from various parts of the plant such as preheating coils, etc., carried with the reactant vapors are often sufficient to cause a serious poisoning of these catalysts. Thus, in general it is found that the activity of these catalysts is decreased approximately linearly from 80% of their initial activity with an iron content of 0.7% to 40% when the iron content is increased to 1.3%. This deactivation of the catalyst, unlike that due to a deposition of tarry materials, is permanent and cannot be counteracted by any of the known regeneration processes. Since these various con-

versions are often executed under pressure, and since furthermore they generally require the introduction or withdrawal of considerable quantities of heat to or from the reaction zone, usually through the confining walls, it is usually impractical in these processes to employ apparatus constructed of or lined with non-ferrous materials such as silica, ceramic materials and the like, and the use of iron, steel or ferrous alloy equipment is practically unavoidable.

The industry has searched diligently for some practical method whereby the transfer of iron to these catalysts could be avoided, while at the same time using apparatus fabricated from ferrous metals. It has, for example, been proposed to employ apparatus plated with chromium, aluminum, copper, etc. Such apparatus sometimes works well for a short time. It is found, however, that these various linings invariably have minute pinholes or become scratched by the catalyst and after a short period of operation the under metal is attacked through these imperfections, with the result that the lining becomes pitted or peels and iron is transferred to the catalyst. The contamination of these catalysts by iron has also been minimized to a considerable extent by the use of certain alloy steels such, in particular, as the more or less corrosion resistant steels containing chromium, nickel, etc. It is found, for example, that whereas iron and plain carbon steels are practically useless, the tendency to contaminate the catalyst with iron is considerably decreased by the incorporation of chromium. However, even chrome steel containing 27% chromium has not proved entirely satisfactory for the purpose. The reaction vessels fabricated from this material are both expensive and relatively short-lived. After a period of use they suddenly begin to contaminate the catalyst with iron and must be discarded. It has also been proposed to employ ferrous metal equipment which has been pretreated with hydrogen sulfide. This pretreatment is sometimes effective in preventing carbon formation in non-catalytic processes, and when employing catalysts which are not susceptible to iron poisoning. It does not, however, avoid or decrease iron contamination and in fact increases it. The pretreatment of the ferrous metal equipment with hydrogen sulfide, when employing catalysts of the above-described type, is furthermore not suitable for use in such processes wherein the catalyst is periodically regenerated as above-described, due to the fact that upon regeneration the coating of protective sulfide formed on the

metal surface by the hydrogen sulfide treatment is destroyed, liberating sulfur dioxide which then poisons the catalyst.

In Patent No. 2,269,028, we have, with George E. Liedholm, described and claimed a simple, practical and effective method whereby the contamination of these catalysts with iron when used in such processes in contact with ferrous metals may be substantially obviated. According to the process of said patent, this is effected by maintaining in the reaction zone certain specified small concentrations of oxygenated sulfur compounds, such in particular as carbonyl sulfide. The desired results may also be obtained according to the method described and claimed in co-pending application Serial No. 391,748, also with George E. Leidholm. According to the process of said co-pending application, iron contamination of the catalyst is prevented by maintaining in the reaction zone small specified concentrations of non-oxygenated sulfur compounds, such in particular as elemental sulfur and thiophenic sulfur compounds.

These processes are very effective in preventing iron contamination of the catalyst. It will be noted, however, that the elemental sulfur or sulfur compound added is found in the product. This, although it is not serious, is disadvantageous in certain instances since for many uses the product must be sulfur-free and this sulfur must be subsequently removed. For example, in the catalytic dehydrogenation of butane to butylene, the butylene is usually polymerized and the polymer hydrogenated to produce iso-octane. For the production of iso-octane by this method, it is desired to have butylene as free from sulfur compounds as possible. One of the advantages of the process of the above-mentioned application over that of the above-mentioned patent is that elemental sulfur and thiophenic sulfur compounds can usually be removed from the product by a relatively simple treatment. Thus, elemental sulfur in the product can be substantially completely removed by thoroughly washing the product with caustic solution. Thiophenic sulfur compounds can usually be substantially completely removed in the case of the treatment of lower boiling hydrocarbons by extraction or by scrubbing with a heavy oil. The recovered thiophenic sulfur compounds can be re-used.

As pointed out, these processes are regenerative, i. e. the catalyst is periodically regenerated in situ by burning carbonaceous deposits therefrom. This necessarily involves subjecting the catalyst and confining converter walls to alternate reducing conditions during the treatment and oxidizing conditions during the regeneration. This alternate changing from reducing to oxidizing and from oxidizing to reducing conditions is particularly prone to cause degradation of ferrous metals and contamination of the catalyst by iron. Under these relatively severe conditions a considerably greater concentration of sulfur or sulfur compounds is required to inhibit iron contamination of the catalyst than would be required if the process were effected continuously under reducing conditions. During the regeneration step most of the effect of the sulfur used in the feed is destroyed.

As shown in the above-mentioned patent and patent application, if the reactant is sulfur-free, iron transfer to the catalyst and catalyst poisoning therefrom are relatively severe. We have now found that the disadvantages arising from the addition of sulfur compounds to the feed may be

eliminated while avoiding iron contamination of the catalyst and at the same time employing a feed which is substantially sulfur-free.

The process of the invention is generally applicable in the conversion of sulfur-free organic or carbonaceous materials in the vapor phase at elevated temperatures at least equal to 500° F. wherein the conversion is executed in ferrous metal reactors with the aid of regenerative catalysts which are affected by contamination by iron. The process is of particular advantage for such of these processes as are endothermic since in these processes the metal confining walls are usually heated and this increases the tendency of the catalyst to become contaminated by iron. Thus, for example, it may be applied for the dehydrogenation of indene to chrysenes, acenaphthene to acenaphthylene, alcohols to aromatic hydrocarbons, isopropyl benzol to methyl styrene, cyclopentane to cyclopentadiene, etc. The process is, however, especially suitable for the dehydrogenation of petroleum hydrocarbons. Thus, it may be advantageously employed for the treatment of any of the common petroleum fractions which are vaporizable without decomposition. Since, however, the more higher boiling of such petroleum fractions usually contain considerable amounts of sulfur compounds, the process will find most application to the treatment of the lighter more nearly sulfur-free fractions such, for example, as the so-called C<sub>2</sub>, C<sub>3</sub>, C<sub>4</sub>, and C<sub>5</sub> fractions. These various materials to be treated, if sulfur-free, can be used per se. If they contain appreciable amounts of sulfur compounds, it is, however, necessary to first submit them to a suitable desulfurization treatment to reduce the sulfur content to within the permissible limit. Any of the conventional desulfurization treatments well known in the art may be used for this purpose. Suitable concentrations of sulfur in the feed to be treated are, for example, from 0 to about 0.0009%.

The various substantially sulfur-free materials are treated under known suitable conditions to effect the desired conversion. Any of the regenerative oxide catalysts can be employed. The process is, however, very effective when employing catalysts of the dehydrogenation type such as the oxides of the metals selected from the left-hand members of Groups IV, V and VI of the Periodic System of the Elements, for example Ti, V, Cr, Mo and W. These various catalytic oxides may, if desired, be employed in admixture with oxides selected from Groups I and/or III. For example, a very suitable catalyst comprises an adsorptive alumina impregnated with 4-20% chromium oxide. Such catalysts are susceptible to poisoning by iron; they are strong dehydrogenation catalysts and are regenerative. In general, when employing catalysts of this type in the vapor phase treatment of the various materials, the temperature of the treatment is between about 500° F. and 1300° F. The use of these catalysts for the treatment of organic materials at these temperatures causes the catalyst to be relatively quickly deactivated by the deposition of carbonaceous deposits thereon. After a relatively short time, for example 2-12 hours, the catalyst activity declines to an uneconomical level. At this point the feed is stopped and an inert gas is passed through the catalyst to flush out residual reactants, and hydrogen, if this is employed in the reaction step. Carbon is next removed from the catalyst by combustion with a stream of an oxygen-containing gas. The gas

employed in this regeneration treatment is usually an inert gas to which air has been added to bring the oxygen concentration to a point where the heat of combustion can be controlled, for example 1%–4%. In some cases pure air may be used. After the carbonaceous deposits have been sufficiently removed, the oxygen-containing gas is flushed from the catalyst with inert gas, and the catalyst is put back on-stream. If hydrogen is recycled in the process, the hydrogen recycle can be initiated prior to starting the feed. This series of steps is repeated at frequent intervals. The inert gas used to flush the catalyst and/or to which oxygen is added to effect the burning is hereinafter referred to as the regeneration gas.

Transfer of iron to the catalyst is inhibited, according to the process of the present invention, by maintaining in the regeneration gas a low and controlled amount of sulfur in the form of sulfur dioxide. It is found that if the regeneration gases contain certain specific concentrations of sulfur dioxide, iron contamination of the catalyst is substantially inhibited even when employing sulfur-free feeds. The concentrations of sulfur dioxide in the regeneration gas employed in the present process must be carefully controlled, however, since insufficient concentrations will not prevent iron contamination of the catalyst and the use of excessive amounts of sulfur dioxide is not only detrimental to the activity of the catalyst but causes severe corrosion. Thus, when employing a substantially sulfur-free feed, i. e., having a sulfur content below about 0.0009%, suitable concentrations of sulfur in the form of sulfur dioxide are between 0.001% and 0.019%. These various points are illustrated in the following examples. These examples, for the sake of comparison, all relate to the dehydrogenation of propane vapors under the following conditions:

Temperature --- 1140° F.

Pressure ----- 1 atm.

Space velocity.. 35 volumes propane at normal conditions per volume catalyst per hour

Catalyst ----- 8-14 mesh pieces of active alumina impregnated with chromium oxide (11% Cr, 0.025% Fe, 0.045% S)

Process period.. 40 min.

The catalyst in each example was employed in a new sand-blasted KA2S steel tube.

#### Example I

Propane vapors substantially free of sulfur were treated under the above-described conditions. After only 19 (and 38) process cycles, i. e. 19 (and 38) 40-minute process periods followed by 19 (and 38) regeneration periods, the catalyst was found to contain about 0.26% iron (and 0.35% iron). In other words, in check runs during 19 and 38 process cycles iron was transferred from the new KA2S steel tube to the catalyst to the extent of about 0.24% (and 0.33%) by weight of the catalyst. It is seen that when the feed is substantially sulfur-free and sulfur dioxide is not added to the regeneration gases, iron transfer to the catalyst is severe even with a new chrome-nickel steel tube.

#### Example II

To the vapors of substantially sulfur-free propane there was added vapors of elemental sulfur

10 to a sulfur content of 0.0045% (and in a similar experiment, 0.006%). The propane vapors containing the specified amounts of elemental sulfur were dehydrogenated under the above-described conditions. During 200 process cycles the iron transfer to the catalyst was in both cases not more than 0.015%. Similar results are obtained with other sulfur compounds in place of elemental sulfur. It is seen that by the application of specific concentrations of sulfur in the feed iron transfer to the catalyst is substantially inhibited. The product, however, contains sulfur which, in most cases, must be removed by a separate treatment.

#### Example III

Substantially sulfur-free propane was dehydrogenated under the above-described conditions. No sulfur or sulfur compound was added to the propane but 0.0007% sulfur in the form of sulfur dioxide was added to the regeneration gas. After only 69 process cycles the tube wall was in very poor condition and the catalyst was found to be severely contaminated with iron (0.10%). It is thus seen that when using a sulfur-free feed a concentration of sulfur dioxide in the regeneration gas equivalent to 0.0007% sulfur is insufficient to prevent iron poisoning of the catalyst.

#### Example IV

Substantially sulfur-free propane was dehydrogenated under the above-described conditions. No sulfur or sulfur compound was added to the propane but 0.005% sulfur in the form of sulfur dioxide was added to the regeneration gas. At the end of 100 process cycles the conversion was 28.2% and at the end of 200 process cycles the conversion was 28.0%. The catalyst at the end of 200 process cycles contained only 0.041% iron (i. e. contamination of only 0.016%). The tube wall was in perfect condition. Thus, it is seen that by the use of 0.005% sulfur in the form of sulfur dioxide in the regeneration gas, iron poisoning of the catalyst is substantially eliminated. Furthermore, since no sulfur is added to the sulfur free feed, the product does not require a subsequent treatment to remove sulfur.

#### Example V

Substantially sulfur-free propane was dehydrogenated under the above-described conditions. No sulfur was added to the propane but 0.025% sulfur in form of sulfur dioxide was added to the regeneration gas. During 193 process cycles 0.20% iron was transferred to the catalyst and the reaction tube was badly corroded. Thus, it is seen that 0.025% sulfur in the form of sulfur dioxide in the regeneration gas does not inhibit iron contamination of the catalyst but, on the other hand, increases it and causes severe corrosion of the chrome-nickel tube.

As explained above and illustrated in the examples, contamination of the catalyst with iron may be substantially inhibited either by the proper application of sulfur or sulfur compounds in the feed according to the above-mentioned patent and co-pending application or according to the present invention, by the use of suitable concentrations of sulfur dioxide in the regeneration gas. It is also possible and often advantageous to apply both of these methods simultaneously. It will be observed, however, that in this case the concentrations of sulfur in both the feed and the regeneration gas are different than when applying either method alone. Thus, according to a

more particular aspect of the present process, a very small and allowable concentration of sulfur is maintained in the feed. Suitable concentrations are between about 0.0009% and 0.0029%, said concentrations being insufficient to effectively prevent iron poisoning of the catalyst. When feeds containing such concentrations of reducible sulfur compounds, such in particular as carbonyl sulfide, elemental sulfur and thiophenic sulfur compounds, are employed, the transfer of iron to the catalyst may be effectively inhibited with smaller concentrations of sulfur dioxide in the regeneration gas. Thus, it is possible to effectively inhibit iron transfer to the catalyst with as low as about 0.0005% sulfur in the regeneration gas. On the other hand, when employing feeds containing between about 0.0009% and 0.0029% sulfur, the maximum concentrations of sulfur dioxide in the regeneration gas which may be effectively employed are lower than when employing sulfur-free feeds. Thus, the maximum concentration of sulfur in the regeneration gas is about 0.01%. In general, the concentrations of sulfur in the feed and in the regeneration gas vary inversely, that is, the higher the concentrations of sulfur in the feed, the lower the concentrations of sulfur dioxide in the regeneration gas. For example, with a feed containing about 0.0006% sulfur a suitable concentration of sulfur in the regeneration gas is about 0.005%, whereas with a feed containing 0.002% the concentration of sulfur in the regeneration gas is preferably about 0.0007%. The application of very small amounts of sulfur in the feed along with the specified concentrations of sulfur dioxide in the regeneration gas, although it does not produce a totally sulfur-free product, produces a product having permissible concentrations of sulfur and is furthermore somewhat more effective in preventing iron poisoning than either method alone.

The sulfur dioxide may be added to the regeneration gas in the desired amounts by simply mixing the desired amount of sulfur dioxide vapors with the regeneration gases entering the regeneration zone. In such cases where the regeneration gases are recycled, for instance according to the method of regeneration claimed in U. S. Patent No. 2,225,402, the sulfur dioxide may be recycled and reused. If desired, however, in order to facilitate control, the regeneration gas may be scrubbed to remove sulfur dioxide and then a measured amount of sulfur dioxide added. Since sulfur dioxide is very cheap and only very small quantities are required, this does not involve any substantial loss.

The contamination of the catalyst by iron in the execution of these various reactions may be inhibited, according to the present process, in the presence of any of the steels and common ferrous alloys. Iron and mild steel are not usually employed in these processes due to their lesser ability to withstand the more or less severe conditions. Particularly suitable materials which may be used are the chrome steels such as KA2, KA2S, KA2ST, KA2Cb, KA2Mo, KA2MoT, etc. In the past these otherwise excellent steels have not been found entirely suitable due to their tendency to cause iron contamination of the catalyst after a short period of use and the industry has been forced to go to the more expensive and difficultly workable high-chrome steel such as 27-Cr, etc. These latter materials, although definitely superior to most low-chrome steels, are nevertheless far from satisfactory and cause iron contamination after a relatively short time. By utilizing the process of the

present invention, any of such steels may be used indefinitely without any appreciable tendency to cause iron contamination of the catalyst. Particularly excellent results are also obtained using nitrogen- or aluminum-stabilized high-chrome steels. For example, a particularly excellent steel has the following composition:

|                | Per cent |
|----------------|----------|
| C              | 0.14     |
| 10 Mn          | 0.40     |
| S              | 0.012    |
| P              | 0.021    |
| Si             | 0.38     |
| Cr             | 26.78    |
| 15 Ni          | Trace    |
| N <sub>2</sub> | 0.17     |

We claim as our invention:

1. In a process for the conversion of carbonaceous materials in the vapor phase at an elevated temperature at least equal to 500° F. wherein the reactant vapors are contacted with a catalyst susceptible to contamination by iron in the presence of a ferrous metal and the catalyst is periodically regenerated in situ by oxidation of carbonaceous deposits therefrom with a stream of regeneration gas of low and controlled oxygen concentration, the step of inhibiting the contamination of the catalyst by iron which comprises maintaining in the feed to the reaction zone less than 0.0009% sulfur and maintaining in the regeneration gas to the regeneration zone between 0.001% and 0.019% sulfur in the form of sulfur dioxide.

2. In a process for the conversion of carbonaceous materials in the vapor phase at an elevated temperature at least equal to 500° F. wherein the reactant vapors are contacted with a dehydrogenating metal oxide catalyst susceptible to contamination by iron in the presence of a ferrous metal and the catalyst is periodically regenerated in situ by oxidation of carbonaceous deposits therefrom with a stream of regeneration gas of low and controlled oxygen concentration, the step of inhibiting the contamination of the catalyst by iron which comprises maintaining in the feed to the reaction zone less than 0.0009% sulfur and maintaining in the regeneration gas to the regeneration zone between 0.001% and 0.019% sulfur in the form of sulfur dioxide.

3. In a process for the conversion of carbonaceous materials in the vapor phase at an elevated temperature at least equal to 500° F. wherein the reactant vapors are contacted with a chromium oxide catalyst in the presence of a ferrous metal and the catalyst is periodically regenerated in situ by oxidation of carbonaceous deposits therefrom with a stream of regeneration gas of low and controlled oxygen concentration, the step of inhibiting the contamination of the catalyst by iron which comprises maintaining in the feed to the reaction zone less than 0.0009% sulfur and maintaining in the regeneration gas to the regeneration zone between 0.001% and 0.019% sulfur in the form of sulfur dioxide.

4. In a process for the conversion of carbonaceous materials in the vapor phase at an elevated temperature at least equal to 500° F. wherein the reactant vapors are contacted with a catalyst susceptible to contamination by iron confined in a chrome steel reactor and the catalyst is periodically regenerated in situ by oxidation of carbonaceous deposits therefrom with a stream of regeneration gas of low and controlled oxygen concentration, the step of inhibiting the con-

tamination of the catalyst by iron which comprises maintaining in the feed to the reaction zone less than 0.0009% sulfur and maintaining in the regeneration gas to the regeneration zone between 0.001% and 0.019% sulfur in the form of sulfur dioxide.

5. In a process for the dehydrogenation of butane in the vapor phase at an elevated temperature at least equal to 500° F. wherein butane vapors are contacted with a dehydrogenating metal oxide catalyst susceptible to contamination by iron in the presence of a ferrous metal and the catalyst is periodically regenerated in situ by oxidation of carbonaceous deposits therefrom with a stream of regeneration gas of low and controlled oxygen concentration, the step of inhibiting the contamination of the catalyst by iron which comprises maintaining in the feed to the reaction zone less than 0.0009% sulfur and maintaining in the regeneration gas to the regeneration zone between 0.001% and 0.019% sulfur in the form of sulfur dioxide.

6. In a process for the dehydrogenation of propane in the vapor phase at an elevated temperature at least equal to 500° F. wherein propane vapors are contacted with a dehydrogenating metal oxide catalyst susceptible to contamination by iron in the presence of a ferrous metal and the catalyst is periodically regenerated in situ by oxidation of carbonaceous deposits therefrom with a stream of regeneration gas of low and controlled oxygen concentration, the step of inhibiting the contamination of the catalyst by iron which comprises maintaining in the feed to the reaction zone less than 0.0009% sulfur and maintaining in the regeneration gas to the regeneration zone between 0.001% and 0.019% sulfur in the form of sulfur dioxide.

7. In a process for the dehydrogenation of butane in the vapor phase at an elevated temperature at least equal to 500° F. wherein the butane vapors are contacted with a chromium oxide catalyst in the presence of a ferrous metal and the catalyst is periodically regenerated in situ by oxidation of carbonaceous deposits therefrom with a stream of regeneration gas of low and controlled oxygen concentration, the step of inhibiting the contamination of the catalyst by iron which comprises maintaining in the feed to the reaction zone less than 0.0009% sulfur and maintaining in the regeneration gas to the regeneration zone between 0.001% and 0.019% sulfur in the form of sulfur dioxide.

8. In a process for the dehydrogenation of propane in the vapor phase at an elevated temperature at least equal to 500° F. wherein the propane vapors are contacted with a chromium oxide catalyst in the presence of a ferrous metal and the catalyst is periodically regenerated in situ by ox-

dation of carbonaceous deposits therefrom with a stream of regeneration gas of low and controlled oxygen concentration, the step of inhibiting the contamination of the catalyst by iron which comprises maintaining in the feed to the reaction zone less than 0.0009% sulfur and maintaining in the regeneration gas to the regeneration zone between 0.001% and 0.019% sulfur in the form of sulfur dioxide.

9. In a process for the conversion of carbonaceous material in the vapor phase at an elevated temperature at least equal to 500° F. wherein the reactant vapors are contacted with a catalyst susceptible to contamination by iron in the presence of a ferrous metal and the catalyst is periodically regenerated in situ by oxidation of carbonaceous deposits therefrom with a stream of regeneration gas of low and controlled oxygen concentration, the step of inhibiting the contamination of the catalyst by iron which comprises maintaining in the feed to the reaction zone between 0.0009% and 0.0029% sulfur and maintaining in the regeneration gas to the regeneration zone between 0.0005% and 0.01% sulfur in the form of sulfur dioxide.

10. In a process for the dehydrogenation of butane in the vapor phase at an elevated temperature at least equal to 500° F. wherein butane vapors are contacted with a dehydrogenating metal oxide catalyst susceptible to contamination by iron in the presence of a ferrous metal and the catalyst is periodically regenerated in situ by oxidation of carbonaceous deposits therefrom with a stream of regeneration gas of low and controlled oxygen concentration, the step of inhibiting the contamination of the catalyst by iron which comprises maintaining in the feed to the reaction zone between 0.0009% and 0.0029% sulfur and maintaining in the regeneration gas to the regeneration zone between 0.0005% and 0.01% sulfur in the form of sulfur dioxide.

11. In a process for the dehydrogenation of propane in the vapor phase at an elevated temperature at least equal to 500° F. wherein propane vapors are contacted with a dehydrogenating metal oxide catalyst susceptible to contamination by iron in the presence of a ferrous metal and the catalyst is periodically regenerated in situ by oxidation of carbonaceous deposits therefrom with a stream of regeneration gas of low and controlled oxygen concentration, the step of inhibiting the contamination of the catalyst by iron which comprises maintaining in the feed to the reaction zone between 0.0009% and 0.0029% sulfur and maintaining in the regeneration gas to the regeneration zone between 0.0005% and 0.01% sulfur in the form of sulfur dioxide.

ROBERT M. COLE.  
IRVING I. SHULTZ.